

# UNITED STATES PATENT OFFICE.

ALFRED L. BROADBENT AND RICHARD G. WOODBRIDGE, JR., OF WILMINGTON, DELAWARE, ASSIGNEES TO E. I. DU PONT DE NEMOURS AND COMPANY, OF WILMINGTON, DELAWARE, A CORPORATION OF DELAWARE.

## PROCESS OF MAKING PROPELLENT POWDER.

1,313,459.

Specification of Letters Patent.

Patented Aug. 19, 1919.

No Drawing.

Application filed July 14, 1916. Serial No. 109,249.

*To all whom it may concern:*

Be it known that we, ALFRED L. BROADBENT and RICHARD G. WOODBRIDGE, Jr., of Wilmington, county of New Castle, State of Delaware, have invented a new and useful Improvement in Processes of Making Propellant Powder, of which the following is a full, clear, and exact description.

Our invention relates to a process of producing explosives of an advantageous character, and more particularly, however, to the production of propellant powders of the progressive type, that is to say which are so treated as to provide a lower initial pressure without reducing the velocity of the projectile. Our invention is applicable to the various kinds of rifle and cannon powders.

A further object is to provide a powder of this type which avoids the great disadvantage present in previous powders of this type due to the fact that said powder comprised coatings on the outside but not impregnating the surface of the powder grain, thus rendering the powder grains so difficult of ignition that hang-fires have resulted unless very strong primers were used.

A further object is to provide a process by means of which the surface of the powder grains may be effectively impregnated with a deterrent in such a manner that the grains are prevented from adhering to each other, and to obtain a more uniform impregnation of the grain by the coating than has heretofore been obtained.

While our invention is capable of embodiment in many different forms, for the purpose of illustration we shall describe only one process indicating the manner in which our invention may be carried out.

For example, we may proceed as follows:

Nitrocellulose powder grains are provided with a coating of a deterrent explosive, such as a nitrohydrocarbon, but preferably, by dinitrotoluene, as, for example, the 1, 2, 4 isomere (c. p. dinitrotoluene), although the mixture of dinitrotoluene as obtained by the direct nitration of toluol may be used. This coating may be applied in the following manner, for example:

The dinitrotoluene may be dissolved in a suitable solvent, as for example benzol, to give a practically saturated solution. The benzol need not be the pure article but may

be the usual commercial grade. The solution of the dinitrotoluene in benzol is made practically saturated simply to save solvent. This solution is sprayed on the powder while the grains are stirred over and over. The solvent may be evaporated as by means of an air blast, leaving the powder grains coated on the surface with the dinitrotoluene. However, we prefer to use the following practice. Instead of dissolving the dinitrotoluene in the benzol and spraying on this solution, we prefer to mix the dinitrotoluene with the grains of powder and then thoroughly wet the powder with the benzol. The amount of benzol required is very much less than that required to completely dissolve the dinitrotoluene. The powder grains are then turned over and over as by revolving the drum or container, and the solvent action of the benzol on the dinitrotoluene is such that within a half hour to an hour, the crystals of dinitrotoluene have practically disappeared. The benzol is then evaporated as by means of an air blast and the powder is found to be coated on the surface with the dinitrotoluene. Or the coating material may be applied in the form of a dry powder by the use of a tumbling barrel, in which the nitrocellulose powder grains and the dinitrotoluene in the form of a dry powder are mixed and subjected to the action of heat sufficient to melt the coating material and cause it to adhere to the powder grains.

The powder grains when coated in this manner are very difficult of ignition, if they are not subjected to the following further treatment, in accordance with our invention: After the powder grains have been provided with the coating of dinitrotoluene, as above, they are immersed in hot water, preferably at a temperature of from 40° to 70° C., depending upon the melting point of the coating compound used. However, it is not necessary to raise the temperature to the melting point of the coating material, because it is sufficiently softened to penetrate the surface of the grains at a temperature somewhat below the melting point. The most advantageous temperature is from 55° to 65° C. for the water bath in which the grains are immersed, although the true melting point of the dinitrotoluene when pure is about 70° C. The powder grains are re-

tained in the bath of hot water for a period of from several hours to several days, but we have found that usually one day is sufficient. The treatment by the hot water causes the deterrent explosive to be absorbed by the powder grains so that while the deterrent explosive is concentrated near the surface of the powder grains it penetrates into the same for a considerable depth, so that in the burning of the powder the successively exposed surfaces contain less and less of the deterrent explosive, thus causing the combustion to proceed with increasing rapidity. We have found that a charge of 15 39.6 grains of colloided nitrocellulose rifle powder, after having been provided with a coating as above described, and dried and glazed with graphite, and without having been subjected to the water treatment, gives 20 a velocity of 2420 feet to a second, and a mean pressure of 48,800 lbs. per square inch. A sample of the same powder, after having been subjected to the water treatment at 60° C. for about fifteen hours, and 25 then dried, when tested with the same rifle, gives the same velocity, but with a mean pressure of only 43,300 lbs.

The hot water performs the functions of applying heat to the coated grains and acting 30 as a medium to keep the grains from adhering to each other. This it does because it is both an agent for applying heat and a fluid which is not a solvent of the coating or of the powder. The two functions might, of 35 course, be separately performed.

While we have described our invention above in detail, we wish it to be understood that many changes may be made therein without departing from the spirit of our 40 invention.

We claim:

1. The process of impregnating the surface of an explosive grain insoluble in water with a deterrent material substantially insoluble in water which comprises subjecting 45 the grain, in contact with said deterrent material, to treatment with hot water.

2. The process which comprises impregnating the surface of an explosive grain insoluble in water with a deterrent explosive substantially insoluble in water by subjecting the grain, coated with said deterrent explosive, to treatment with hot water.

3. The process which comprises impregnating the surface of an explosive grain insoluble in water with a dinitrotoluene by subjecting the grain, coated with said dinitrotoluene, to treatment with hot water.

4. The process which comprises impregnating the surface of an explosive grain insoluble in water with a substantially pure 1-2-4 dinitrotoluene by subjecting the grain, coated with said substantially pure 1-2-4 dinitrotoluene, to treatment with hot 65 water.

5. The process which comprises impregnating the surface of an explosive grain insoluble in water with a dinitrotoluene by subjecting the grains intimately mixed with said dinitrotoluene, to treatment with hot 70 water.

6. The process which comprises impregnating the surface of an explosive grain insoluble in water with substantially pure 1-2-4 dinitrotoluene by subjecting the grains, 75 intimately mixed with said substantially pure 1-2-4 dinitrotoluene, to treatment with hot water.

7. The process which comprises impregnating the surface of an explosive grain insoluble in water with a deterrent material substantially insoluble in water by subjecting the grains, intimately mixed with the 80 said deterrent material, to treatment with hot water.

8. The process which comprises impregnating the surface of an explosive grain insoluble in water with a deterrent explosive substantially insoluble in water by subjecting the grains, intimately mixed with the 85 said deterrent explosive, to treatment with hot water.

9. The process which comprises impregnating the surface of an explosive grain insoluble in water with a deterrent material substantially insoluble in water by subjecting the grain, coated with said deterrent material, to treatment with hot water at a temperature below the melting point of the coating 95 material.

10. The process which comprises impregnating the surface of an explosive grain insoluble in water with a deterrent explosive substantially insoluble in water by subjecting the grain, coated with said deterrent explosive, to treatment with hot water at a temperature below the melting point of the coating material.

11. The process which comprises impregnating the surface of an explosive grain insoluble in water with a dinitrotoluene by subjecting the grain, coated with said dinitrotoluene, to treatment with hot water at a temperature below the melting point of the coating material.

12. The process which comprises impregnating the surface of an explosive grain insoluble in water with a substantially pure 1-2-4 dinitrotoluene, by subjecting the grain, coated with said dinitrotoluene, to treatment with hot water, at a temperature below the melting point of the coating material.

13. The process which comprises impregnating the surface of a nitrocellulose powder grain with a deterrent material substantially insoluble in water by subjecting the grain, coated with said deterrent material, to treatment with hot water.

14. The process which comprises impregnating

nating the surface of a nitrocellulose powder grain with a deterrent explosive substantially insoluble in water by subjecting the grain, coated with said deterrent explosive, 5 to treatment with hot water.

15. The process which comprises impregnating the surface of a nitrocellulose powder grain with a dinitrotoluene by subjecting the grain, coated with said dinitrotoluene, 10 to treatment with hot water.

16. The process which comprises impregnating the surface of a nitrocellulose powder grain with a substantially pure 1-2-4 dinitrotoluene by subjecting the grain, coated 15 with said substantially pure 1-2-4 dinitrotoluene, to treatment with hot water.

17. The process which comprises impregnating the surface of a nitrocellulose powder grain with a deterrent material substantially 20 insoluble in water by subjecting the grain, coated with said deterrent material, to treatment with hot water at a temperature below the melting point of the coating material.

18. The process which comprises impregnating the surface of a nitrocellulose powder grain with a deterrent explosive substantially insoluble in water by subjecting the grain, coated with said deterrent explosive, 25 to treatment with hot water at a temperature below the melting point of the coating material.

19. The process of impregnating the surface of powder grains with a deterrent material insoluble in water, while preventing 35 the grains from adhering, comprising subjecting powder grains coated with the deterrent material to a treatment with hot water.

20. The process of impregnating the surface of powder grains with a deterrent material, while preventing the grains from adhering, comprising subjecting powder grains 40 coated with a deterrent explosive material substantially insoluble in water to a treatment with water heated below the melting point of the coating material.

21. The process which comprises coating a powder grain with a deterrent material, subjecting the coated grain to an inert liquid heating medium to melt the deterrent 50 material and maintaining the coated grain in contact with said heating medium until the deterrent material has substantially impregnated the grain.

22. The process which comprises coating a powder grain with a deterrent explosive, subjecting the coated grain to an inert liquid heating medium to melt the deterrent explosive, and maintaining the coated grain 55 in contact with said heating medium until the deterrent explosive has substantially impregnated the grain.

23. The process which comprises coating a powder grain with a dinitrotoluene, subjecting the coated grain to an inert liquid heating medium to melt the dinitrotoluene, 60

and maintaining the coated grain in contact with said heating medium until the dinitrotoluene has substantially impregnated the grain.

24. The process which comprises coating 70 a powder grain with a substantially pure 1-2-4 dinitrotoluene, subjecting the coated grain to an inert liquid heating medium to melt the dinitrotoluene, and maintaining the coated grain in contact with said heating 75 medium until the dinitrotoluene has substantially impregnated the grain.

25. The process of impregnating the surface of explosive powder grains with a deterrent material which comprises agitating 80 the powder grains in the presence of the deterrent material and a volatile solvent of the deterrent material, evaporating the solvent to leave a coating on the grains, and subjecting the resulting coated grains to water 85 sufficiently hot to melt the coating.

26. The process which comprises coating and impregnating the surface of explosive grains with a deterrent material, and subjecting the coated grains to the action of 90 heat and a liquid medium to keep the grains from adhering to each other.

27. The process which comprises coating and impregnating the surface of explosive powder grains with a deterrent explosive, 95 and subjecting the grains to the action of heat and a liquid which is not a substantial solvent of the coating or of the powder.

28. The process which comprises coating and impregnating the surface of a nitrocellulose powder grain with a dinitrotoluene, and subjecting the coated grains to the action of 100 heat and of a liquid medium to keep the grains from adhering to each other.

29. The process which comprises coating 105 and impregnating the surface of a nitrocellulose powder grain with a substantially pure 1-2-4 dinitrotoluene, and subjecting the grains to the action of heat and of a liquid medium which is not a substantial solvent of the coating or of the powder.

30. That step in the process of impregnating the surface of an explosive powder grain with a deterrent material comprising agitating the powder grain in the presence of a 115 dry deterrent material and adding a less quantity of volatile solvent than will form a saturated solution of the deterrent material and evaporating the solvent to leave a coating on the grain.

31. That step in the process of impregnating the surface of an explosive powder grain with dinitrotoluene comprising agitating the powder grain in the presence of dinitrotoluene and benzol and evaporating the benzol 125 to leave a coating of dinitrotoluene on the powder grain.

32. That step in the process of impregnating the surface of an explosive powder grain with dinitrotoluene comprising agitating the 130

powder grain in the presence of dinitrotoluene and benzol in a less quantity than is necessary to form a saturated solution of the dinitrotoluene and evaporating the solvent 5 to leave a dinitrotoluene coating on the grain.

In testimony whereof we have hereunto set our hands at Wilmington, county of New

Castle, State of Delaware, on the days and dates opposite our names written.

ALFRED L. BROADBENT. July 7, 1916.

RICHARD G. WOODBRIDGE, JR. July 7, 1916.

Witnesses:

A. M. GORMAN,

P. E. STRICKLAND.